# EUROPEAN PATENT SPECIFICATION

(11) **EP 1 238 157 B1**
(45) Date of publication and mention of the grant of the patent: **11.06.2008**
(21) Application number: 00966911.0
(22) Date of filing: 26.09.2000
(51) Int. Cl.: D21H 19/38, B41M 5/00, C09D 5/03

(54) **RECORDING MEDIUM**
AUFZEICHNUNGSMEDIUM
SUPPORT D'ENREGISTREMENT

(30) Priority: 01.10.1999 US 157462 P
(43) Date of publication of application: 11.09.2002
(62) Divisional of application: 08008392.6
(73) Proprietor: CABOT CORPORATION, Boston, Massachusetts 02210-2019 (US)
(72) Inventor: DARSILLO, Michael, S., Clifton Park, NY 12065 (US); FLUCK, David, J., Bel Aire, MD 21015 (US); LAUFHUTTE, Rudiger, Tuscola, IL 61953 (US)
(74) Representative: Trueman, Lucy Petra
(86) International application number: PCT/US2000/026464
(87) International publication number: WO 2001/025534

(56) References cited:
- EP-A- 0 878 322
- EP-A- 1 048 479
- US-A- 5 171 626
- US-A- 5 472 773
- US-A- 5 527 423
- US-A- 5 679 451
- PATENT ABSTRACTS OF JAPAN vol. 1999, no. 14, 22 December 1999 (1999-12-22) & JP 11 246218 A (ASAHI GLASS CO LTD), 14 September 1999 (1999-09-14)

## Description

### TECHNICAL FIELD OF THE INVENTION

The present invention relates to recording media comprising alumina particles in the coating thereof, compositions comprising such particles, and production methods therefor.

### BACKGROUND OF THE INVENTION

A surface coating is sometimes applied to a recording medium in order to improve its printing properties. For example, the coating can improve the appearance, ink absorption, and/or image smear resistance of the medium.

Surface coatings can be classified into two general categories -- glossy coatings and non-glossy (matte or dull) coatings. Glossy coatings are highly desirable, as they are very smooth, and can impart a superior feel and a photograph-like quality to a recorded image. However, it remains a challenge to provide a glossy medium that imparts superior printing properties to the medium (e.g., good ink absorption, good dye-fixing ability, good waterfastness, and/or good resistance to image smear), in addition to superior smoothness and gloss.

Gloss and dye immobilization (i.e., dye-fixing) can sometimes be achieved by incorporating different types of polymeric resins into a coating. For example, a gelatin, a polyvinyl alcohol, a polyolefin resin, polyester resin, polyamide resin, and/or polycarbonate resin can be used to produce glossiness, while a cationic polymer (e.g., polyvinylpyrrolidone) can be used to promote the surface immobilization of an anionic dye. However, inks applied to resin-coated recording media dry relatively slowly, and often have an undesirable tendency to smear and rub off. While some pigments such as certain treated kaolin clays or treated calcium carbonates can immobilize dyes, the overall absorptivity and rate of absorption are often compromised.

Using a metal oxide pigment such as silica or alumina can be advantageous in that they have good absorptivity and also can produce an excellent coating. Alumina is particularly advantageous in that its particles naturally have a cationic surface (i.e., a positive zeta potential) Since the vast majority of ink dyes are anionic in nature, the cationic surface of alumina imparts superior dye immobilizing properties to coatings derived therefrom. Moreover, alumina also imparts good ink absorption, good waterfastness, and good image smear resistance, in addition to superior gloss, smoothness, and brightness, to the coating.

US 5,171,626 describes an ink-jet recording medium comprising a substrate and a pigment layer, with the pigment layer comprising an upper layer and a lower layer. The upper layer contains as a major pigment an aluminium oxide having a specific surface area ranging from 90 m²/g to 170 m²/g. The lower layer may contain as a major pigment an aluminium oxide having a specific surface area that is smaller than the aluminium oxide in the upper layer.

EP-A-0 878 322 describes an ink-jet recording material having high glass, which comprises an under recording layer and an upper recording layer, each of these layer comprising pigment having an average secondary particle size of 10 to 400 nm and a binder, with the pigment preferably being selected from silica, alumina, silicate, alumina and calcium carbonate pigments, with amorphous silica being particularly preferred.

Despite its advantages, the use of alumina presents significant challenges in the recording medium coating industry in that alumina is very difficult to process. Unlike silica, which is typically amorphous, alumina is crystalline, and can exist in various crystalline phases, for example, alpha, or the transitional phases, for example, gamma, delta, and theta phases. In addition, long drying times are typically required in recording medium coating which utilize low solids alumina dispersions, making the overall coating process costly and inefficient. Moreover, some forms of alumina require a relatively high binder ratio (about 3:1 pigment to binder ratio). The high binder demand of alumina restricts the ratio of alumina particles (relative to binder) that can be achieved in the coating, sacrificing desirable properties that could otherwise be imparted to the coating by the alumina particles (e.g., drying time, dye immobilization, waterfastness, image quality, and the like). As such, the overall quality of the recording medium can be limited.

Poor colloidal stability of alumina also seriously limits the solids content that can be attained in coating compositions used to make the recording media, thereby placing an upper limit on coater productivity (throughput), as drier demand can be excessive in order to adequately dry the coating on the substrate. In a commercial setting, such coating compositions are produced from an initial alumina dispersion. The initial dispersion is often manufactured in a separate facility and shipped to the end user. Typically, the end user processes the initial dispersion into a coating composition, which is normally applied to a substrate shortly after its production.

As dispersions with higher alumina solids content have a greater tendency to gel or separate (i.e., the solid settles out of the dispersion), low solids initial dispersions are used. As such, the overall quality of recording media is limited by the low alumina solids content (e.g., in terms of porosity, dye immobilization, image quality, or the like).

Accordingly there remains a need for an improved recording medium comprising alumina particles, desirably having a low binder demand and high porosity, as well as an alumina-based coating composition and a method of producing such a composition and recording medium. The present invention provides such a recording medium, coating composition, and methods of making them. These and other advantages of the present invention, as well as additional inventive features, will be apparent from the description of the invention provided herein.

### BRIEF SUMMARY OF THE INVENTION

The present invention provides an ink-jet recording medium comprising a substrate having a glossy coating thereon, wherein the glossy coating has a 75° specular gloss of about 15% or more comprises a binder and alumina particles that are aggregates of primary particles. The coating of the recording medium of the present invention comprises alumina particles that are aggregates of primary particles which are pyrogenic or fumed alumina particles having a surface area of 30-80 m²/g.

The present invention further provides a coating composition comprising fumed alumina particles and a binder, wherein the alumina particles have a surface area of 30-80 m²/g and the solids content of the fumed alumina particles in the coating composition is 10 to 50 wt.%.

The present invention also provides a method of preparing a coating composition. The inventive method of preparing a coating composition comprises providing a colloidally stable dispersion comprising water and fumed alumina particles having a surface area of 30-80 m²/g and the solids content of the fumed alumina particles in the dispersion is 20 to 50 wt.%; adding a binder to and, optionally, diluting the colloidally stable dispersion, until a desired pigment to binder ratio and overall solids content are obtained; and optionally adjusting the pH with a suitable acid or base.

The present invention additionally provides a method of preparing a recording medium. The inventive method of preparing a recording medium comprises providing a substrate; coating the substrate with the coating composition of the present invention to produce a substrate coated with a coating; optionally calendering the coated substrate; and drying the coated substrate.

The coating composition of the present invention dries quickly when applied to a substrate, to form a non-tacky glossy coating.

### DESCRIPTION OF THE PREFERRED EMBODIMENTS

The present invention provides a recording medium comprising a substrate having a glossy coating thereon, wherein the glossy coating comprises a binder and alumina particles that are aggregates of primary particles.

The inventive recording medium comprises a substrate, which can be either transparent or opaque, and which can be made of any suitable material. Examples of such materials include, but are not limited to, films or sheets of polymer resins (e.g., poly(ethylene terephthalate)), diacetate resins, triacetate resins, acrylic resins, polycarbonate resins, polyvinyl chloride resins, polyimide resins, cellophane and celluloid, glass sheets, metal sheets, plastic sheets, paper (e.g., cellulose paper, synthetic paper), coated paper (e.g., resin-coated paper), pigment-containing opaque films, and foamed films. Polyester sheets and cellulose paper are preferred, with poly(ethylene terephthalate) sheets being a preferred polyester.

The substrate used in the recording medium of the present invention has a glossy coating thereon, which,can be of any suitable thickness. In particular, the coating is preferably from 1 µm to 50 µm in thickness, more preferably from 5 µm to 40 µm in thickness, and most preferably from 10 µm to 30 µm in thickness. The recording medium of the present invention provides excellent gloss and also has good ink absorption, dye immobilization, a high rate of liquid absorption, and overall liquid absorption capacity. Moreover, the recording medium of the present invention provides excellent image quality, particularly when used in ink jet printing applications.

In certain embodiments of the present invention the inventive recording medium comprises a substrate having more than one layer of coating, which can be the same or different. However, at least one of the coating layers comprises alumina particles with properties as described herein. For example, the recording medium of the present invention can comprise a substrate coated with one or more ink-receptive layers (e.g., comprising anionic silica) and/or one or more resinous layers (e.g., a glossy, laminated surface layer). Even when the recording medium of the present invention comprises such additional layers of coating, it has been found that the above-described glossy coating comprising the alumina particles described herein provides sufficient ink absorption, dye immobilization, and gloss for the vast majority of printing applications.

The coating of the recording medium of the present invention comprises alumina particles that are aggregates of primary particles which are pyrogenic or fumed alumina particles. Particles of pyrogenic alumina are aggregates of smaller, primary particles. Although the primary particles are not porous, the aggregates contain a significant void volume, and are capable of rapid liquid absorption. These void-containing aggregates enable a coating to retain a significant capacity for liquid absorption even when the aggregate particles are densely packed, which minimizes the inter-particle void volume of the coating.

The size of the alumina particles of which the coating is comprised impacts the glossiness of the coating. It should be noted that when the alumina particles used in the present invention comprise aggregates of fused (i.e., aggregated) primary particles, the diameter values refer to the diameters of the aggregates. Particle diameter can be determined by any suitable technique, for example, by a light scattering technique, (e.g., using a Brookhaven 90Plus Particle Scanner, available from Brookhaven Instruments Corporation, Holtsville, New York).

In order to maximize glossiness, it is preferred that the mean diameter of the alumina particles (i.e., the aggregates) is less than 1 µm. More preferably, the mean diameter of the alumina particles is less than 500 nm, still more preferably the mean diameter of the alumina particles is less than 400·nm, and most preferably the mean diameter of the alumina particles is less than 300 nm.

It is highly preferred that at least 80% (e.g., at least 90%) or substantially all of the alumina particles have diameters smaller than the mean diameter values set forth above. In other words, it is highly preferred that at least 80% (e.g., at least 90%) or substantially all of the particles have diameters of less than about 1 µm, more highly preferred that at least 80% (e.g., at least 90%) or substantially all of the particles have diameters of less than 500 nm, still more highly preferred that at least 80% (e.g., at least 90%) or substantially all of the particles have diameters of less than 400 nm, and most highly preferred that at least 80% (e.g., at least 90%) or substantially all of the particles have diameters of less than 300 nm.

In certain preferred embodiments, the mean diameter of the alumina particles is at least 40 nm (e.g., particles having a mean diameter from 40 nm to 300 nm, preferably from 80 nm to 300 nm, more preferably from 100 nm to 200 nm, still more preferably from 120 to 190 nm, and most preferably from 140-180 nm (e.g., from 150-170 nm)). In certain of these embodiments, at least 80% (e.g., at least 90%) or substantially all of the alumina particles have diameters of at least 100 nm (e.g., from 100 nm to 200 nm, more preferably from 120 to 190 nm, and most preferably from 140-180 nm (e.g., from 150-170 nm)).

In other embodiments of the present invention, the alumina particles preferably have a mean diameter of less than 300 nm, more preferably less than 200 nm, still more preferably less than 190 nm, and most preferably less than 180. In certain embodiments it is preferred that at least 80% (e.g., at least 90%) or substantially all of the alumina particles have diameters of less than 300 nm, more preferably less than 200 nm, still more preferably less than 190 nm, and most preferably less than 180 nm.

The coating can comprise alumina particles having any suitable range of individual particle diameters, such as a relatively broad range or a relatively narrow range. The particles also can be monodispersed. By monodispersed is meant that the individual particles have diameters that are substantially identical. For example, substantially all monodispersed 150 nm particles have diameters in the range of from 140 nm to 160 nm.

With respect to the primary particles that make up these alumina aggregates, in certain embodiments of the present invention, such as when a glossy coating having a relatively high rate of and capacity for liquid absorption is desired, it is preferred that the primary particles have a mean diameter of less than 100 nm (e.g., from 1 nm to 100 nm). More preferably, the primary particles have a mean diameter of less than 80 nm (e.g., from 1 nm to 80 nm), even more preferably less than 50 nm (e.g., from 1 nm to 50 nm), and most preferably less than 40 nm (e.g., from 5 nm to 40 nm).

In certain of these embodiments it is preferred that at least 80% (e.g., at least 90%) or substantially all of the primary particles have diameters smaller than the mean diameter values set forth above. In other words, it is preferred that at least 80% (e.g., at least 90%) or substantially all of the primary particles have diameters of less than 100 nm (e.g., from 1 nm to 100 nm), more preferred that at least 80% (e.g., at least 90%) or substantially all of the primary particles have diameters of less than 80 nm (e.g., from 1 nm to 80 nm), even more preferred that at least 80% (e.g., at least 90%) or substantially all of the primary particles have diameters of less than 50 nm (e.g., from 1 nm to 50 nm), and most preferred that at least 80% (e.g., at least 90%) or substantially all of the primary particles have diameters of less than 40 nm (e.g., from 5 nm to 40 nm).

It will be appreciated that the surface area of the alumina particles of the recording medium of the present invention is largely a function of the mean diameter of the primary particles, rather than the mean diameter of the aggregates. The alumina particles of the recording medium of the present invention can have a surface area of 30-80 m²/g. The alumina particles of the recording medium of the present invention most preferably have a surface area of 40-60 m²/g.

The glossiness of the recording medium of the present invention can be measured using any suitable technique. For example, the glossiness of the present invention can be measured in terms of the 75° specular gloss according to JIS P 8142, or an equivalent U.S. standard, using a gloss photometer, for example, a VGS-1001, manufactured by Nihon Denshoku Kogyosha, a Hunter 75° Gloss Meter, a Technidyne Glossmeter (e.g., Model T480A), or the like. Other suitable test methods can be used to determine glossiness, for example, ASTM, TAPPI, or the like. When TAPPI is used, it is preferably TAPPI T480. When ASTM is used, it is preferably ASTM D1223.

The recording medium of the present invention has a 75° specular gloss of at least 15%. More preferably, the recording medium of the present invention has a glossiness of at least 25%, even more preferably at least 35%, still more preferably at least 45%. In some instances, the glossiness is least 55%, and even at least 65%.

Desirably, the recording medium of the present invention is calendered to provide a glossier coating. The recording medium, when calendered preferably has a 75° specular gloss of at least 15%, more preferably at least 25%, even more preferably at least 35%, and still more preferably at least 45%. In a preferred embodiment, the recording medium of the present invention, when calendered, has a 75° specular gloss of at least 50%. In some instances, depending on the substrate, the coating compostion, the nature of the coating composition, and the method of applying the coating to the substrate, the recording medium of the present invention, when calendered, can have glossiness is least 55%, and even at least 65%.

The coating of the recording medium of the present invention has good dye immobilization properties and waterfastness. Organic dyes, such as those used in ink-jet inks, often contain ionizable functional groups (e.g., SO₃H, COOH, PO₃H₂, etc.), which increase the water solubility of the dyes. The dyes become negatively charged when these functional groups ionize in water (e.g., to SO₃⁻, COO⁻, PO₃²⁻, etc.). As the alumina used in the glossy coating of the recording medium of the present invention has a cationic surface, the alumina particles enhances the ability of the coating to immobilize (i.e., adsorb) and display dye molecules at the surface of the coating. This is due to the strong electrostatic attraction of the dye toward the alumina particles in the glossy coating of the recording medium of the present invention.

Therefore, even though the ink can be rapidly absorbed into the coating via the pores of the alumina particles, the anionic dye molecules can be separated from the ink, and immobilized at the coating surface. As such, the coating of the recording medium of the present invention has excellent dye immobilizing ability, which promotes desirable qualities, for example, superior image quality and high optical density.

It is desirable for the alumina particles in the coating of the the recording medium of the present invention to have a high positive zeta potential. The net charge on the alumina particles of the recording medium of the present invention can be qualitatively determined by measuring the zeta potential of the dispersion (e.g., using a Matec MBS 8000 or a Brookhaven Zeta Plus instrument). A negative zeta potential is indicative of a net negative charge, while a positive zeta potential indicates a net positive charge. The magnitude of the zeta potential is proportional to the magnitude of the charge.

Dye adhesion to the surface of a recording medium can be quantified by measuring the optical density and waterfastness of a test sample of the recording medium to which an aqueous ink-jet ink comprising an anionic dye has been applied. For example, a test sample having an ink coverage of about 12 g/m² over an area of about 90 cm² can be cut in half and tested in the following manner. One minute after applying the ink, one of the halves is soaked in deionized water for one minute and then repeatedly dipped in and out of the water to remove all dissolved ink from the sample. After drying, a densitometer (e.g., a MacBeth 512 densitometer) can be used to measure the image intensity at a number of positions (e.g., at ten random positions) on each half of the test sample, and the values for each half averaged. The optical density of the recording medium is the average image intensity of the half of the test sample that was not soaked in water. The waterfastness can be reported as: $1 - \left[\frac{\left(ave. I.I. of unsoaked)-(ave. I.I. of soaked\right)}{\left(ave. I.I. of unsoaked\right)}\right]$
wherein ave. I.I. is the average image intensity of each half of the test sample (i.e., the half that was soaked in water and the half that was not soaked in water). Waterfastness values that are less than one, when calculated in this fashion, generally indicate loss of ink from the coating.

Alternatively, waterfastness can be evaluated in terms of retained optical density. For example, a test print can be evaluated by immersing a sample in deionized water for 5 minutes with light agitation, drying the sample, and comparing the color density of the dry soaked sample with that of an unsoaked sample (as indicated above) by measuring color density with a suitable densitomer (e.g., X-Rite^{®} 938 Spectrodensitometer). Waterfastness can then be expressed in terms of the percentage of optical density retained by the soaked sample relative to the unsoaked sample.

The recording medium of the present invention exhibits excellent waterfastness. For example, the recording medium of the present invention typically retains at least about 50% of the optical density after immersion in deionized water for 5 minutes with light agitation. Preferably, after it is immersed in deionized water for 5 minutes with light agitation, the recording medium of the present invention retains at least 60% of the optical density of the printed image, more preferably at least 70% of the optical density, still more preferably at least 80% of the optical density, and most preferably at least 90% of the optical density is retained (e.g., 95% or even 100% of the optical density).

The recording medium of the present invention also has a good rate of liquid absorption and good capacity for liquid absorption. The rate of liquid absorption can be measured by any suitable method, for example, by applying a droplet of a liquid (e.g., distilled water) to the coating surface and measuring the change in the angle of the droplet with respect to the surface (contact angle) over time. Preferably, the contact angle of distilled water, when applied to the glossy coating of the recording medium of the present invention, decreases by at least 5° over the first five minutes. More preferably, the contact angle decreases by at least 7° over the first five minutes. Most preferably, the contact angle of distilled water, when applied to the glossy coating of the recording medium of the present invention, decreases by at least 10° over the first five minutes.

The capacity for liquid absorption of the coating of the recording medium of the present invention can be measured by any suitable technique. For example, the capacity for liquid absorption can be measured by contacting a liquid, for example, water, or a 1:1 solution of polyethylene glycol (e.g., PEG 400) and water, or the like, with a predetermined area of the glossy coating of the recording medium of the present invention for 10 seconds at 22 °C, followed by contacting the medium with a blotting paper to remove excess solution, measuring the weight of the solution absorbed by the glossy coating, and expressing that weight in terms of g/m².

Alternatively, the liquid absorption capacity of the coating can be measured as a function of porosity. Porosity can be measured by any suitable method, for example, by measuring the total intrusion volume of a liquid (e.g., mercury) into the glossy coating applied to a non-porous substrate (e.g., polyethylene). It will be appreciated that the total intrusion volume of a liquid for a particular coating (and, therefore, the porosity) can be a function of variables that influence the structure of the coating, for example, binder type, pigment-to-binder ratio, pigment particle size, calendering, and the like. Preferably, the porosity is determined by measuring the total intrusion volume of mercury. In this regard, the glossy coating of the recording medium of the present invention, when the substrate is a non-porous substrate, preferably has a total mercury intrusion volume of at least 0.3 ml/g, more preferably at least 0.5 ml/g, still more preferably at least 0.8 ml/g, most preferably 1 ml/g or greater.

The properties of the inventive recording medium promote high image quality when used in the vast majority of printing applications. Any suitable printing method can be used to apply an image to the inventive recording medium. Such printing methods include, but are not limited to gravure, letterpress, collotype, lithography (e.g., offset lithography), ink-jet, and printing with hand-held implements (e.g., pens), with ink-jet printing being preferred.

Any suitable binder can be used in the coating of the recording medium of the present invention. Preferred binders include, but are not limited to, polyvinyl alcohol (PVOH), polyvinyl acetate, polyvinyl acetal, polyvinyl pyrrolidone, oxidized starch, etherified starch, cellulose derivatives (e.g., carboxymethyl cellulose (CMC), hydroxyethyl cellulose, etc.), casein, gelatin, soybean protein, silyl-modified polyvinyl alcohol, conjugated diene copolymer latexes (e.g., maleic anhydride resin, styrene-butadiene copolymer, methyl methacrylate-butadiene copolymers, etc.), acrylic polymer latexes (e.g., polymers and copolymers of acrylic esters and methacrylic esters, polymers and copolymers of acrylic acid and methacrylic acid, etc.), vinyl polymer latexes (e.g., ethylene-vinyl acetate copolymer), functional group-modified polymer latexes obtained by modifying the above-mentioned various polymers with monomers containing functional groups (e.g., carboxyl groups), aqueous binders such as thermosetting resins (e.g., melamine resin, urea resin, etc.), synthetic resin binders such as polymethyl methacrylate, polyurethane resin, polyester resin (e.g., unsaturated polyester resin), amide resin, vinyl chloride-vinyl acetate copolymer, polyvinyl butyral, and alkyd resin, with polyvinyl alcohol being most preferred.

The alumina particles in the coating of the recording medium of the present invention have a low binder demand. As such, a higher pigment to binder ratio can be utilized in the coating of the recording medium of the present invention. The high pigment to binder ratio is advantageous in that a greater number of alumina particles per unit volume can exist in the coating of the recording medium of the present invention, improving the properties thereof (e.g., gloss and porosity). Preferably, the pigment to binder ratio of the coating of the recording medium of the present invention is at least 2:1 by weight. More preferably the pigment to binder ratio of the coating of the recording medium of the present invention is at least 5:1 by weight, still more preferably at least 7:1 by weight, and most preferably at least 8:1 by weight. In some embodiments, the pigment to binder ratio of the coating of the recording medium of the present invention is at least 9:1 by weight (e.g., at least 10:1 by weight).

The total amount of binder (i.e., dry binder) can be any suitable amount, but is preferably from 1% to 50% of the composition (i.e., dry binder and particles combined) by weight. More preferably, the total amount of binder is from 1% to 40% of the composition by weight, even more preferably from 1% to 30% by weight, still more preferably from 3% to 25% by weight, yet more preferably from 5% to 15% by weight, and most preferably from 5% to 10% by weight (e.g., 9% by weight).

When PVOH is used as a binder, the total amount of PVOH is preferably from 1% to 50% of the composition by weight, more preferably from 1% to 40% by weight, even more preferably from 1% to 30% by weight, yet more preferably from 3% to 25% by weight, still more preferably from 5% to 15% by weight, and most preferably from 5% to 10% by weight (e.g., 9% by weight).

In certain embodiments of the present invention, the glossy coating of the inventive recording medium comprises one or more pigments in addition to fumed alumina particles, such as calcium carbonate, clays, aluminum silicates, urea-formaldehyde fillers, and the like. Other suitable pigments include silica (e.g., colloidal silica, precipitated silica, silica gel, pyrogenic silica, or cationically modified analogs thereof), alumina (e.g., alumina sols, colloidal alumina, cationic aluminum oxide or hydrates thereof, pseudoboehmite, boehmite, Al(OH)₃, etc.), magnesium silicate, magnesium carbonate, kaolin, talc, calcium sulfate, barium sulfate, titanium dioxide, zinc oxide, zinc sulfide, zinc carbonate, satin white, diatomaceous earth, calcium silicate, aluminum hydroxide, lithopone, zeolite, hydrated halloycite, magnesium hydroxide, polyolefins (e.g., polystyrene, polyethylene, polypropylene, etc.), plastics (e.g., acrylic), urea resin, and melamine resin.

The glossy coating of the recording medium of the present invention also can comprise one or more other additives, such as surfactants (e.g., cationic surfactants, anionic surfactants such as long-chain alkylbenzene sulfonate salts and long-chain, preferably branched chain, alkylsulfosuccinate esters, nonionic surfactants such as polyalkylene oxide ethers of long-chain, preferably branched-chain alkyl group-containing phenols and polyalkylene oxide ethers of long-chain alkyl alcohols, and fluorinated surfactants), silane coupling agents (e.g., γ-aminopropyltriethoxysilane, N-β (aminoethyl) γ-aminopropyltrimethoxysilane, etc.), hardeners (e.g., active halogen compounds, vinylsulfone compounds, aziridine compounds, epoxy compounds, acryloyl compounds isocyanate compounds, etc.), pigment dispersants, thickeners (e.g., carboxymethyl cellulose (CMC)), flowability improvers, antifoamers (e.g., octyl alcohol, silicone-based antifoamers, etc.), foam inhibitors, releasing agents, foaming agents, pentetrants, coloring dyes, coloring pigments, whiteners (e.g., fluorescent whiteners), preservatives (e.g., p-hydroxybenzoate ester compounds, benzisothiazolone compounds, isothiazolone compounds, etc.), antifungal agents, yellowing inhibitors (e.g., sodium hydroxymethanesulfonate, sodium p-toluenesulfinate, etc.), ultraviolet absorbers (e.g., benzotriazole compounds having a hydroxy-dialkylphenyl group at the 2-position), antioxidants (e.g., sterically hindered phenol compounds), antistatic agents, pH regulators (e.g., sodium hydroxide, sodium carbonate, sulfuric acid, hydrochloric acid, phosphoric acid, citric acid, etc.), water-resisting agents, wet strengthening agents, and dry strengthening agents.

The present invention further provides a coating composition comprising fumed alumina particles and a binder, wherein the alumina particles have a surface area of 30-80 m²/g and the solids content of the alumina in the coating composition is 10 to 50 wt.%.

Any suitable fumed alumina particles can be used in the coating composition of the present invention. Suitable alumina particles include the alumina particles described herein with respect to the coating of the recording medium of the present invention. The alumina particles used in the coating composition of the present invention can be of any suitable diameter and have a surface area of 30-80 m²/g. Suitable particle diameters and surface areas of the particles include the particle diameters and surface areas described herein with respect to the coating of the recording medium of the present invention.

Any suitable binder can be used in coating composition of the present invention, including those described herein with respect to the coating of the recording medium of the present invention. Likewise, any suitable pigment to binder ratio can be used in the coating composition of the present invention. Preferably, the pigment to binder ratio is at least 2:1 by weight. More preferably the pigment to binder ratio of the coating composition of the present invention is at least 5:1 by weight, still more preferably at least 7:1 by weight, and most preferably at least 8:1 by weight. In some embodiments, the pigment to binder ration of the coating composition of the present invention is at least 9:1 by weight (e.g., at least 10:1 by weight).

The coating composition of the present invention typically includes a suitable carrier. The carrier can be any suitable fluid or combination of fluids (e.g., solvents) in which the first and second groups of particles, and any other additives (e.g., one or more binders), can be mixed and applied to a substrate. Preferred carriers have a relatively high vapor pressure to accelerate drying of the coating after application, and preferred examples include, but are not limited to, organic solvents (e.g., methanol) and water, with water being most preferred.

In certain embodiments, coating composition of the present invention comprises one or more pigments in addition to fumed alumina particles, including those described herein with respect to the coating of the recording medium of the present invention. The coating composition of the present invention also can comprise one or more other additives, for example, surfactants, silane coupling agents, hardeners, pigment dispersants, thickeners, flowability improvers, antifoamers, foam inhibitors, releasing agents, foaming agents, pentetrants, coloring dyes, coloring pigments, whiteners, antifungal agents, yellowing inhibitors, ultraviolet absorbers, antioxidants, water-resisting agents, wet strengthening agents, and dry strengthening agents, including those described herein with respect to the coating of the recording medium of the present invention.

The present invention further provides a method of preparing a coating composition. The method comprises:
providing a colloidally stable dispersion comprising water and fumed alumina particles, wherein the fumed alumina particles have a surface area of 30-80 m²/g and the solids content of the alumina particles in the dispersion is at 20 to 50 wt.%;
adding a binder to and, optionally, diluting the colloidally stable dispersion, until a desired pigment to binder ratio and overall solids content are obtained; and
optionally adjusting the pH with a suitable acid or base.

Any suitable fumed alumina particles can be used in the inventive method of preparing a coating composition. Suitable alumina particles include the alumina particles described herein with respect to the coating of the recording medium of the present invention. The alumina particles used in the inventive method of preparing a coating composition can be of any suitable diameter and have a surface area of 30-80 m²/g. Suitable particle diameters and surface areas of the particles include the particle diameters and surface areas described herein with respect to the coating of the recording medium of the present invention.

Any suitable binder can be used in the inventive method of preparing a coating composition, including those described herein with respect to the coating of the recording medium of the present invention. Likewise, any suitable pigment to binder ratio can be used in preparing the coating composition in accordance with the method of the present invention. Preferred pigment to binder ratios include those described herein with respect to the coating of the recording medium of the present invention.

A suitable carrier can be employed in the method of preparing a coating composition of the present invention. The carrier can be present in the dispersion or can be added to the dispersion to produce the final coating composition. Suitable carriers include those described herein with respect to the coating of the recording medium of the present invention, with water being most preferred.

In accordance with the inventive method of preparing a coating composition, one or more pigments can be added to the dispersion in addition to the alumina particles, including those described herein with respect to the coating of the recording medium of the present invention. One or more other additives also can be added, including those described herein with respect to the coating of the recording medium of the present invention.

The colloidally stable dispersion (i.e., the initial dispersion) used to prepare the coating composition in accordance with the present invention has a high solids content (i.e., greater than 20 wt.% alumina solids) and also is colloidally stable. The high alumina solids content of the initial dispersion is highly advantageous in that a higher solids content of the coating composition can be achieved (e.g., at least 20 wt.% total solids taking the binder and other additives into account). As a result, drying time in coating operations is significantly diminished, making the overall process less costly and more efficient. The initial dispersion can be prepared by any suitable method, but is preferably prepared according to the method described in U-S. Patent 5,527,423.

Preferably, the alumina solids content of the initial dispersion is at least 25 wt.%, more preferably at least 30 wt.%, still more preferably at least 35 wt.%, even more preferably at least 40 wt.%, and most preferably al least 50 wt.%. In certain embodiments, the alumina solids content of the colloidally stable dispersion is 25-50 wt. % or 30-50 wt.%, but is more preferably 30-50 wt.%, most preferably 40-50 wt.%.

The alumina particles in the initial dispersion used in the method of the present invention can have any suitable positive zeta potential. Desirably, the positive zeta potential is sufficiently high to promote colloidal stability in the initial dispersion. Preferably, the zeta potential of the alumina particles in the initial dispersion is at least +20 mV. More preferably, the zeta potential of the alumina particles in the initial dispersion dispersion is at least +30 mV. Most preferably, the zeta potential of the alumina particles in the initial dispersion dispersion is at least +40 mV.

The initial dispersion can be of any suitable pH. Preferably, the pH of the initial dispersion is 3-5, and more preferably is 3.5-4.5, but most preferably is 4-4.5. While the initial dispersion can have a range of specific gravity values, the specific gravity of the initial dispersion preferably is in the range of 1-2 kg/l.

The initial dispersion used to prepare the coating composition of the present invention has excellent rheological properties, making the dispersion and coating compositions derived therefrom highly amenable to large scale coating operations. For example, the initial dispersion exhibits low viscosity at a high shear rate, e.g., as measured in a Hercules® High-Shear Viscometer at 4400 RPM, FF Bob measuring geometry. Preferably, the initial dispersion, at an alumina solids content of about 40 wt.%, has an apparent viscosity of less than 0.02 Pa.s (20 cp) at high shear rate (e.g., as measured in a Hercules® High-Shear Viscometer at 4400 RPM, FF Bob measuring geometry). More preferably, the initial dispersion (at about 40 wt.% alumina solids) has an apparent viscosity of less than 0.015 Pa.s (15 cp), as measured in a Hercules® High-Shear Viscometer at 4400 RPM, FF Bob measuring geometry. Most preferably, the initial dispersion (at about 40 wt.% alumina solids) has an apparent viscosity of less than 0.01 Pa.s (10 cp), as measured in a Hercules® High-Shear Viscometer at 4400 RPM, FF Bob measuring geometry,

The initial dispersion used to prepare the coating composition of the present invention also exhibits low viscosity at a low shear rate, e.g., as measured in a Brookfield Model RV viscometer, spindle #1, after about 30 seconds at 60 RPM. Preferably, the initial dispersion (at about 40 wt.% alumina solids) has an apparent viscosity of less than 0.1 Pa.s (100 cp) at low shear rate (e.g., as measured in a Brookfield Model RV viscometer, spindle #1, after about 30 seconds at 60 RPM). More preferably, the initial dispersion (at about 40 wt.% alumina solids) has an apparent viscosity of less than 0.08 Pa.s (80 cp), as measured in a Brookfield Model RV viscometer, spindle #1, after about 30 seconds at 60 RPM. Most preferably, the initial dispersion (at about 40 wt.% alumina solids) has an apparent viscosity of less than 0.05 Pa.s (50 cp), as measured in a Brookfield Model RV viscometer, spindle #1, after about 30 seconds at 60 RPM.

The initial dispersion used to prepare the coating composition of the present invention can be very high in alumina solids content (e.g., 30-50 wt.% alumina solids), yet maintain long-term colloidal stability (e.g., 1 year). Coating compositions prepared from the initial dispersion in accordance with the method of the present invention have a significantly lower binder demand and have greater runnability than conventional alumina coating compositions. Moreover, when applied to a substrate as a coating, the coating composition prepared from the initial dispersion in accordance with the present invention require significantly less drying time than conventional coatings. The coatings on the recording media thus produced have high porosity, excellent gloss, dye-immobilizing ability, and waterfastness, and provide superior image quality.

The present invention further provides a method of preparing a recording medium. The inventive method of preparing a recording medium comprises:
providing a substrate;
coating the substrate with the coating composition of the present invention to produce a substrate coated with a coating;
optionally calendering the coated substrate; and
drying the coated substrate.

As indicated above, the coating composition of the present invention provides fast drying times, drying quickly to form a non-tacky glossy coating. The coating composition can be applied using any suitable method or combination of methods. Suitable methods include, but are not limited to, roll coating, blade coating, air knife coating, rod coating, bar coating, cast coating, gate roll coating, wire bar coating, short-dowel coating, slide hopper coating, curtain coating, flexographic coating, gravure coating, Komma coating, size press coating in the manner of on- or off-machine, and die coating, with rapid, inexpensive methods such as rod coating and air knife coating being preferred.

The coated substrate can be dried using any suitable method. Suitable drying methods include, but are not limited to, air or convection drying (e.g., linear tunnel drying, arch drying, air-loop drying, sine curve air float drying, etc.), contact or conduction drying, and radiant-energy drying (e.g., infrared drying and microwave drying).

Many physical properties of a glossy coating prepared with the coating composition of the present invention, can be rationally optimized by varying the relative quantity of particles from each group contained therein. It will be appreciated that materials other than the alumina particles (e.g., binders, thickeners, and the like) can be varied to alter or optimize the physical properties of the coating composition of the present invention.

The primary features of the inventive method of preparing a recording medium are as previously described with respect to the recording medium and coating composition of the present invention. For example, the preferred substrates, coating methods, coating composition (e.g., solids content, binder content, apparent density, additives, etc.), properties of the alumina particles (i.e., materials, diameters, surface area, etc.), coating properties (i.e., thickness, number and constitution of coating layers, glossiness, rate and capacity of liquid absorption, packing density, adhesiveness, etc.), are as described herein with respect to the recording medium and coating composition of the present invention.

The following examples further illustrate the present invention but, of course, should not be construed as in any way limiting its scope.

### Example 1

This example illustrates the preparation of a coating composition of the present invention. An initial dispersion of fumed alumina was prepared in accordance with U.S. Patent 5,527,423. The fumed alumina had a surface area of about 55 m²/g. The fumed alumina was greater than 95% crystalline, of which about 70% was theta phase, about 20% was delta phase, and about 10% was gamma phase, the fraction of alpha phase having been below the detection limit.

The dispersion had an alumina solids content of 40.0 wt.%, a pH of 4-4.4, and a specific gravity of 1.4 kg/l. The viscosity of the final dispersion was less than 0.05 Pa.s (50 cp) when measured using a Brookfield Model LV viscometer, spindle #1, after 60 seconds at 60 RPM. The mean diameter of the alumina particles in the final dispersion was 154 nm as measured in a Brookhaven 90Plus Particle Scanner (Brookhaven Instruments Corporation, Holtsville, New York).

The initial dispersion had excellent rheological properties. The apparent viscosity of the initial dispersion, as measured in a Hercules® High-Shear viscometer at 4400 RPM, FF Bob measuring geometry, was 0.0088 Pa.s (8.8 cp (centipoise)).

The zeta potential of the particles in the dispersion was +40 mV. The dispersion was colloidally stable in that there was no appreciable increase in viscosity or gellation after one year at a storage temperature ranging from 40-110 °F (4-43 °C).

A coating composition was prepared by adding sufficient polyvinyl alcohol binder (PVOH) to the initial dispersion to give a pigment to binder ratio of 7:1, HEC (1.55 wt.%), and diluting to an overall solids content (including binder) of 24.28 wt.%. The final pH was 4.20. The coating composition had excellent rheological properties. The viscosity of the composition was 0.888 Pa.s (888 cp) when measured using a Brookfield Model RV viscometer, spindle #5, after 30 seconds at 100 RPM. The apparent viscosity of the composition was 0.024 Pa.s (24.1 cp) as measured in a Hercules® High-Shear Viscometer at 4400 RPM, FF Bob measuring geometry.

The coating composition produced excellent coatings with an unusually low pigment to binder ratio of 7:1. The coating composition prepared in this example had significantly lower binder demand than conventional alumina coating compositions, which typically use a 3:1 pigment to binder ratio.

### Example 2

This example illustrates a coating composition prepared from the initial dispersion prepared in Example 1. A coating composition was prepared by adding sufficient polyvinyl alcohol binder (PVOH) to the dispersion prepared in Example 1 to give a pigment to binder ratio of 7:1, and diluting to an overall solids content (including binder) of 22.27 wt.%. The pH was adjusted to about 7.97 with ammonium hydroxide.

The coating composition had excellent rheological properties. The viscosity of the composition was 2.076 Pa.s (2076 cp) when measured using a Brookfield Model RV viscometer, spindle #5, after 30 seconds at 100 RPM. The apparent viscosity of the composition was 0.014 Pa.s (14.0 cp) as measured in a Hercules® High-Shear Viscometer at 4400 RPM, FF Bob measuring geometry.

The coating composition produced excellent coatings with low pigment to binder ratio of 7:1. The coating composition prepared in this example had a low binder demand.

### Example 3

This example illustrates the preparation of a recording medium of the present invention. An uncoated paper substrate base was coated with the coating composition of Example 1, except that the coating composition had a total solids content of 26.3 wt.%, no HEC added was added, the pH of the coating composition was 4.45, and the pigment to binder ratio was 4:1. Coating was performed on a CLC (Cylindrical Laboratory Coater) blade coating apparatus at high speed. The CLC simulates conditions that are characteristic of commercial manufacture. The performance of a particular coating composition in the CLC at high speed is indicative of how the coating composition is expected to perform under high speed commercial manufacturing conditions. The coating was preformed at a rate of 2000 feet per minute (610 meters per minute) using a flexible blade, and the coating was dried (infrared). The coating dried quickly.

The dry coat weight in grams per square meter (g/m²) for each recording medium (i.e., coated substrate) was determined, and the dry recording media (uncalendered) were analyzed. Optical and surface properties were measured for each recording medium and also for the uncoated substrate.

Samples were calendered on one side with 3 nips at 6 pli (pounds per linear inch) (1.25 kg/linear cm) and 60 °C. The optical, surface and printing properties were measured for the calendered samples, and the results were compared to the uncalendered samples.

The uncoated paper substrate had the following properties: basis weight: 77.5 g/m²; pH: 6.6; ash: 8.31%; caliper 3.62/1000" (91.9 µm); brightness: 82.7%; gloss: 6.4%; smoothness: 3.93 µm; Hercules^{®} sizing test: 109 sec; and PPS porosity: 2.77 ml/min. The recording media obtained by coating the substrate in accordance with this example had excellent gloss, brightness, and porosity. The coating had an excellent appearance and superior feel, and did not crack or exhibit brittleness. Moreover, the recording media produced an excellent printed image.

Brightness was measured using a Technidyne^{®} Brightness Meter Tappi Procedure T 452 OM-92. Gloss was measured using a Hunter 75° degree gloss meter according to TAPPI standard procedure T 4800M-92. The surface smoothness and porosity of the sheets were measured using a Parker Print Surf (PPS) tester (TAPPI T555 PM-94). The rate of liquid absorption of the papers was measured using a First 10 Angstrom Dynamic Contact Angle measuring device.

The properties of the recording media (uncalendered and calendered) are shown below in Table 1.

**Table 1**

| Medium | Brightness (%) | 75° Specular Gloss (%) | PPS Smoothness (µm) | Porosity (ml/min.) |
|---|---|---|---|---|
| Uncoated Substrate | 82.7 | 6.4 | 3.93 | 2.77 |
| | | | | |
| Coated Substrate | 86.7 | 13.0 | 3.68 | 82.6 |
| (8 g/m²) | | | | |
| | | | | |
| Calendered | 83.9 | 66.3 | 1.16 | 20.0 |
| (8 g/m²) | | | | |

The samples were printed on Epson Stylus^{®} Pro Photorealistic and Hewlett Packard^{®} 820C ink jet printers using a test pattern created with ADOBE^{®} software. The print gloss and print density of the samples was then measured. Print gloss was measured using a Gardener 60 degree Micro-Gloss meter. Print density was measured using a BYK Gardner^{®} densitometer. The properties of the image as printed using the Epson^{®} Stylus Pro Photorealistic and the Hewlett Packard^{®} 820C are shown in Tables 2A and 2B, respectively.

**Table 2A**

| | Epson Stylus^{®} Pro ES Wide Format | | | | | |
|---|---|---|---|---|---|---|
| Medium | Black | Cyan | Magenta | Yellow | Ink Gloss | Coating Gloss |
| Coated Substrate | 1.44 | 0.69 | 0.91 | 0.79 | 1.82 | 13.0 |
| (8 g/m²) | | | | | | |
| | | | | | | |
| Calendered | 1.64 | 0.73 | 1.02 | 0.98 | 14.8 | 66.3 |
| (8 g/m²) | | | | | | |

**Table 2B**

| | Hewlett Packard^{®} 820C | | | | | |
|---|---|---|---|---|---|---|
| Medium | Black | Cyan | Magenta | Yellow | Ink Gloss | Coating Gloss |
| Coated Substrate | 1.57 | 1.18 | 1.23 | 0.86 | 9.40 | 13.0 |
| (8 g/m²) | | | | | | |
| | | | | | | |
| Calendered | 1.64 | 0.73 | 1.02 | 0.98 | 11.7 | 66.3 |
| (8 g/m²) | | | | | | |

These results demonstrate that the recording media produced in accordance with this example exhibited excellent optical, physical, and textural properties, as indicated by the high measured values for gloss (low PPS smoothness), and the high measured values for brightness and porosity. These results also demonstrate the excellent quality of printed images attainable using such recording media, as indicated by the high values for ink density using several representative colors, as well as high ink gloss values.

### Example 4

Using the CLC apparatus described in Example 3, one side of a cellulose paper substrate was coated with the composition prepared according to Example 1, except that the total solids content of the coating composition was 26.4 wt.%, the pH was 4.5, the amount of HEC added was 3.0 wt.%, and the pigment to binder ratio was 5:1. Coating was performed at a rate of 3000 feet per minute (914 meters per minute) and the samples dried (infrared). The coatings were applied at three different coating weights, and the coatings dried quickly after they were applied to the substrate.

The dry coat weight in grams per square meter (g/m²) for each recording medium was determined, and the dry recording media (uncalendered) were analyzed. Optical and surface properties were measured for each recording medium and also for the uncoated substrate. PPS (Parker Print Surf) roughness and brightness were measured. Brightness was measured in accordance with TAPPI brightness standard. Glossiness was measured in terms of the 75° specular gloss according to JIS P 8142 using a gloss photometer.

The recording media were calendered, and the 75° specular gloss measurements were determined for the calendered media. The results are shown in Table 3.

**Table 3**

| Coat Wt. | Brightness | 75° Specular Gloss | PPS Smoothness | PPS Porosity |
|---|---|---|---|---|
| (g/m²) | (%) | (%) [Calendered] | (uncalendered) | (uncalendered) |
| | | | (µm) | (ml/min) |
| 5.67 | 92.6 | 26.1 **[N/A]** | 4.4 | 69.2 |
| | | | | |
| 7.59 | 91.9 | 21.74 **[69.6]** | 4.2 | 70.6 |
| | | | | |
| 10.85 | 92.2 | 24.92 **[N/A]** | 4.3 | 67.4 |

These data demonstrate that the coating composition of the present invention exhibits excellent performance at high speed and produces a glossy recording medium with excellent optical and surface properties under such conditions. These data demonstrate that the composition of the present invention possesses rheological properties desirable for producing high quality coatings under high speed manufacturing operations.

### Example 5

Using the CLC apparatus described in Example 3, one side of a cellulose paper substrate was coated with the composition prepared according to Example 1, except that the total solids content of the coating composition was 33.3 wt.%, the pH was 4.5, the amount of HEC added was 3.0 wt.%, and the pigment to binder ratio was 5:1. Coating was performed at a rate of 3000 feet per minute (914 meters per minute) and the samples dried (infrared). The coatings were applied at three different coating weights, and the coatings dried quickly after they were applied to the substrate.

The dry coat weight in grams per square meter (g/m²) for each recording medium was determined, and the dry recording media (uncalendered) were analyzed. Optical and surface properties were measured for each recording medium and also for the uncoated substrate. PPS (Parker Print Surf) roughness and brightness were measured. Brightness was measured in accordance with TAPPI brightness standard. Glossiness was measured in terms of the 75° specular gloss according to JIS P 8142 using a gloss photometer.

The recording media were calendered, and the 75° specular gloss measurements were determined for the calendered media. The results are shown in Table 4.

**Table 4**

| Coat Wt. | Brightness | 75° Specular Gloss | PPS Smoothness | PPS Porosity |
|---|---|---|---|---|
| (g/m²) | (%) | (%) [Calendered] | (uncalendered) | (uncalendered) |
| | | | (µm) | (ml/min) |
| 5.00 | 85.1 | 18.0 **[N/A]** | 4.2 | 17.1 |
| | | | | |
| 14.4 | 86.9 | 20.6 **[69.4]** | 4.3 | 20.1 |
| | | | | |
| 15.0 | 86.9 | 22.0 **[N/A]** | 4.3 | 18.3 |
| | | | | |
| 18.0 | 85.1 | 19.80 **[N/A]** | 4.3 | 17.5 |

These data demonstrate that the coating composition of the present invention exhibits excellent performance at high speed and produces a glossy recording medium with excellent optical and surface properties under such conditions. These data demonstrate that the composition of the present invention possesses rheological properties desirable for producing high quality coatings under high speed manufacturing operations.

### Example 6

This example illustrates the rate of liquid absorption of the recording medium of the present invention. A coating composition was prepared in accordance with Example 1 (pigment to binder ratio 7:1), except that the coating composition had a total solids content of 29 wt.%, the pH of the composition was 4.5, and the amount of HEC added was 3.0 wt.%. Recording media were prepared by coating a cellulose paper substrate using the CLC coating apparatus as described in Example 4, except that the applied coating weights were 5.3 g/m², 8.0 g/m², and 13.6 g/m², respectively.

The change in contact angle (for a distilled water droplet) was measured over time for recording medium samples of each coating weight.

Each sample exhibited a sharp initial decrease over the first few minutes, indicating a good rate liquid absorption for a range of coating weights.

## Claims

1. An ink-jet recording medium comprising a substrate having a glossy coating thereon, the glossy coating comprising fumed alumina particles and a binder, wherein the glossy coating has a 75° specular gloss of 15% or more, and the fumed alumina particles are aggregates of primary particles and have a surface area of 30-80 m²/g.

2. The ink-jet recording medium of claim 1, wherein the substrate comprises a polymer or cellulose paper.

3. The ink-jet recording medium of claim 1 or 2, wherein the substrate comprises poly(ethylene terephthalate).

4. The ink-jet recording medium of any of claims 1-3, wherein the aggregates have a mean diameter of less than 1 µm.

5. The ink-jet recording medium of claim 4, wherein the aggregates have a mean diameter of 80-300 nm.

6. The ink-jet recording medium of claim 5, wherein the aggregates have a mean diameter of 100-200 nm.

7. The ink-jet recording medium of claim 4, wherein at least about 80% of the aggregates have a diameter of less than 1 µm.

8. The ink-jet recording medium of claim 7, wherein at least about 90% of the aggregates have a diameter of less than 1 µm.

9. The ink-jet recording medium of any of claims 1-8, wherein the primary particles have a mean diameter of 1-100 mn.

10. The ink-jet recording medium of claim 9, wherein the primary particles have a mean diameter of 1-80 nm.

11. The ink-jet recording medium of claim 10, wherein the primary particles have a mean diameter of 1-50 nm.

12. The ink-jet recording medium of claim 11, wherein the primary particles have a mean diameter of 5-40 nm.

13. The ink-jet recording medium of claim 9, wherein at least about 80% of the primary particles have a diameter of 1-100 nm.

14. The ink-jet recording medium of claim 10, wherein at least about 80% of the primary particles have a diameter of 1-80 nm.

15. The ink-jet recording medium of claim 11, wherein at least about 80% of the primary particles have a diameter of 1-50 nm.

16. The ink-jet recording medium of claim 12, wherein at least about 80% of the primary particles have a diameter of 5-40 nm.

17. The ink-jet recording medium of any of claims 1-16, wherein the alumina to binder ratio is at least 2:1 by weight.

18. The ink-jet recording medium of claim 17, wherein the alumina to binder ratio is 7:1 by weight or more.

19. The ink-jet recording medium of claim 18, wherein the alumina to binder ratio is 9:1 by weight or more.

20. The ink-jet recording medium of any of claims 1-19, wherein the fumed alumina particles have a surface area of 40-60 m²/g.

21. The ink-jet recording medium of any of claims 1-20, wherein the glossy coating has a 75° specular gloss of 65% or more.

22. The ink-jet recording medium of any of claims 1-21, wherein the substrate is non-porous, and the glossy coating has a total mercury intrusion volume of 0.3 ml/g or more.

23. The ink-jet recording medium of claim 22, wherein the glossy coating has a total mercury intrusion volume of 0.8 ml/g or more.

24. A coating composition comprising fumed alumina particles and a binder, wherein the fumed alumina particles are aggregates of primary particles and have a surface area of 30-80 m²/g, and the solids content of the fumed alumina particles in the composition is 10-50 wt.%.

25. The coating composition of claim 24, wherein the aggregates have a mean diameter of less than 1 µm.

26. The coating composition of claim 25, wherein the aggregates have a mean diameter of 80-300 nm.

27. The coating composition of claim 26, wherein the aggregates have a mean diameter of 100-200 nm.

28. The coating composition of any of claims 24-27, wherein the primary particles have a mean diameter of 1-100 nm.

29. The coating composition of claim 28, wherein the primary particles have a mean diameter of 1-80 nm.

30. The coating composition of claim 29, wherein the primary particles have a mean diameter of 1-50 nm.

31. The coating composition of claim 30, wherein the primary particles have a mean diameter of 5-40 nm.

32. The coating composition of any of claims 24-31., wherein the alumina to binder ratio is at least 2:1 by weight.

33. The coating composition of claim 32, wherein the alumina to binder ratio is at least 7:1 by weight.

34. The coating composition of claim 33, wherein the alumina to binder ratio is at least 9:1 by weight.

35. The coating composition of any of claims 24-34, wherein the fumed alumina particles have a surface area of 40-60 m²/g.

36. A method of preparing a coating composition, the method comprising:
providing a colloidally stable dispersion comprising water and fumed alumina particles, wherein the fumed alumina particles are aggregates of primary particles, have a surface area of 30-80 m²/g, and the solids content of the fumed alumina particles in the dispersion is 20-50 wt.%;
adding a binder to and, optionally, diluting the colloidally stable dispersion, until a desired pigment to binder ratio and overall solids content are obtained; and
optionally adjusting the pH with a suitable acid or base.

37. The method of claim 36, wherein the aggregates have a mean diameter of less than 1 µm.

38. The method of claim 37, wherein the aggregates have a mean diameter of 80-300 nm.

39. The method of claim 38, wherein the aggregates have a mean diameter of 100-200 nm.

40. The method of any of claims 36-39, wherein the primary particles have a mean diameter of 1-100 nm.

41. The method of claim 40, wherein the primary particles have a mean diameter of 1-80 nm.

42. The method of claim 41, wherein the primary particles have a mean diameter of 1-50 nm.

43. The method of claim 42, wherein the primary particles have a mean diameter of 5-40 nm.

44. The method of any of claims 36-43, wherein the alumina to binder ratio is at least 2:1 by weight.

45. The method of claim 44, wherein the alumina to binder ratio is at least 7:1 by weight.

46. The method of claim 45, wherein the alumina to binder ratio is at least 9:1 by weight.

47. The method of any of claims 36-46, wherein the fumed alumina particles have a surface area of 40-60 m²/g.

48. The method of any of claims 36-47, wherein the solids content of the fumed alumina particles in the colloidally stable dispersion is 30-50 wt.%.

49. The method of any of claims 36-48, wherein the zeta potential of the alumina particles in the colloidally stable dispersion is at least +20 mV.

50. The method of any of claims 36-49, wherein the pH of the colloidally stable dispersion is 3-5.

51. The method of any of claims 36-50, wherein the specific gravity of the colloidally stable dispersion is 1-2 kg/l.

52. The method of any of claims 36-51, wherein the apparent viscosity of the colloidally stable dispersion is less than 0.02Pa.s (20 cp) as measured in a Hercules^{®} High-Shear Viscometer at 4400 RPM, FF Bob measuring geometry.

53. The method of any of claims 36-53, wherein the viscosity of the colloidally stable dispersion is less than 0.1Pa.s (100 cp) as measured in a Brookfield Model RV viscometer, spindle #1, after 30 seconds at 60 RPM.

54. A coating composition obtainable by the method of any of claims 36-53.

55. A method of preparing an ink-jet recording medium, the method comprising:
providing a substrate;
coating the substrate with the coating composition of any of claims 24-35 to produce a substrate coated with a coating;
optionally calendering the coated substrate; and
drying the coated substrate.

56. A method of preparing an ink-jet recording medium, the method comprising:
providing a substrate;
coating the substrate with the coating composition of claim 54, to produce a substrate coated with a coating;
optionally calendering the coated substrate; and
drying the coated substrate.

57. An ink-jet recording medium obtainable by the method of claim 55 or 56.

## Patentansprüche

1. Tintenstrahlaufzeichnungsmedium, umfassend ein Substrat, das eine glänzende Beschichtung aufweist, wobei die glänzende Beschichtung hochdisperse Aluminiumoxidpartikel und ein Bindemittel umfasst, wobei die glänzende Beschichtung bei 75 ° einen Spiegelglanz von 15 % oder mehr aufweist und die hochdispersen Aluminiumoxidpartikel Aggregate von Primärpartikeln sind und eine Oberfläche von 30 - 80 m² / g aufweisen.

2. Tintenstrahlaufzeichnungsmedium nach Anspruch 1, wobei das Substrat ein Polymer oder Cellulosepapier umfasst.

3. Tintenstrahlaufzeichnungsmedium nach Anspruch 1 oder 2, wobei das Substrat Poly(ethylenterephthalat) umfasst.

4. Tintenstrahlaufzeichnungsmedium nach einem der Ansprüche 1 - 3, wobei die Aggregate einen mittleren Durchmesser von weniger als 1 µm aufweisen.

5. Tintenstrahlaufzeichnungsmedium nach Anspruch 4, wobei die Aggregate einen mittleren Durchmesser von 80 - 300 nm aufweisen.

6. Tintenstrahlaufzeichnungsmedium nach Anspruch 5, wobei die Aggregate einen mittleren Durchmesser von 100 - 200 nm aufweisen.

7. Tintenstrahlaufzeichnungsmedium nach Anspruch 4, wobei mindestens etwa 80 % der Aggregate einen Durchmesser von weniger als 1 µm aufweisen.

8. Tintenstrahlaufzeichnungsmedium nach Anspruch 7, wobei mindestens etwa 90 % der Aggregate einen Durchmesser von weniger als 1 µm aufweisen.

9. Tintenstrahlaufzeichnungsmedium nach einem der Ansprüche 1 - 8, wobei die Primärpartikel einen mittleren Durchmesser von 1 - 100 nm aufweisen.

10. Tintenstrahlaufzeichnungsmedium nach Anspruch 9, wobei die Primärpartikel einen mittleren Durchmesser von 1 - 80 nm aufweisen.

11. Tintenstrahlaufzeichnungsmedium nach Anspruch 10, wobei die Primärpartikel einen mittleren Durchmesser von 1 - 50 nm aufweisen.

12. Tintenstrahlaufzeichnungsmedium nach Anspruch 11, wobei die Primärpartikel einen mittleren Durchmesser von 5 - 40 nm aufweisen.

13. Tintenstrahlaufzeichnungsmedium nach Anspruch 9, wobei mindestens etwa 80 % der Primärpartikel einen Durchmesser von 1- 100 nm aufweisen.

14. Tintenstrahlaufzeichnungsmedium nach Anspruch 10, wobei mindestens etwa 80 % einen Durchmesser von 1 - 80 nm aufweisen.

15. Tintenstrahlaufzeichnungsmedium nach Anspruch 11, wobei mindestens etwa 80 % der Primärpartikel einen Durchmesser von 1 - 50 nm aufweisen.

16. Tintenstrahlaufzeichnungsmedium nach Anspruch 12, wobei mindestens etwa 80 % der Primärpartikel einen Durchmesser von 5 - 40 nm aufweisen.

17. Tintenstrahlaufzeichnungsmedium nach einem der Ansprüche 1-16, wobei das Verhältnis von Aluminiumoxid zu Bindemittel, bezogen auf das Gewicht, mindestens 2:1 beträgt.

18. Tintenstrahlaufzeichnungsmedium nach Anspruch 17, wobei das Verhältnis von Aluminiumoxid zu Bindemittel, bezogen auf das Gewicht, 7:1 oder mehr beträgt.

19. Tintenstrahlaufzeichnungsmedium nach Anspruch 18, wobei das Verhältnis von Aluminiumoxid zu Bindemittel, bezogen auf das Gewicht, 9:1 oder mehr beträgt.

20. Tintenstrahlaufzeichnungsmedium nach einem der Ansprüche 1-19, wobei die hochdispersen Aluminiumoxidpartikel eine Oberfläche von 40 - 60 m² / g aufweisen.

21. Tintenstrahlaufzeichnungsmedium nach einem der Ansprüche 1 - 20, wobei die glänzende Beschichtung bei 75 ° einen Spiegelglanz von 65 % oder mehr aufweist.

22. Tintenstrahlaufzeichnungsmedium nach einem der Ansprüche 1 - 21, wobei das Substrat nicht-porös ist und die glänzende Beschichtung ein Quecksilberintrusionsgesamtvolumen von 0,3 ml / g oder mehr aufweist.

23. Tintenstrahlaufzeichnungsmedium nach Anspruch 22, wobei die glänzende Beschichtung ein Quecksilberintrusionsgesamtvolumen von 0,8 ml / g oder mehr aufweist.

24. Beschichtungszusammensetzung, umfassend hochdisperse Aluminiumoxidpartikel und ein Bindemittel, wobei die hochdispersen Aluminiumoxidpartikel Aggregate von Primärpartikeln sind und eine Oberfläche von 30 - 80 m² / g aufweisen und der Feststoffgehalt der hochdispersen Aluminiumoxidpartikel in der Zusammensetzung 10 - 50 Gew. % beträgt.

25. Beschichtungszusammensetzung nach Anspruch 24, wobei die Aggregate einen mittleren Durchmesser von weniger als 1 µm aufweisen.

26. Beschichtungszusammensetzung nach Anspruch 25, wobei die Aggregate einen mittleren Durchmesser von 80 - 300 nm aufweisen.

27. Beschichtungszusammensetzung nach Anspruch 26, wobei die Aggregate einen mittleren Durchmesser von 100 - 200 nm aufweisen.

28. Beschichtungszusammensetzung nach einem der Ansprüche 24 - 27, wobei die Primärpartikel einen mittleren Durchmesser von 1 - 100 nm aufweisen.

29. Beschichtungszusammensetzung nach Anspruch 28, wobei die Primärpartikel einen mittleren Durchmesser von 1 - 80 nm aufweisen.

30. Beschichtungszusammensetzung nach Anspruch 29, wobei die Primärpartikel einen mittleren Durchmesser von 1 - 50 nm aufweisen.

31. Beschichtungszusammensetzung nach Anspruch 30, wobei die Primärpartikel einen mittleren Durchmesser von 5 - 40 nm aufweisen.

32. Beschichtungszusammensetzung nach einem der Ansprüche 24 - 31, wobei das Verhältnis von Aluminiumoxid zu Bindemittel, bezogen auf das Gewicht, mindestens 2:1 beträgt.

33. Beschichtungszusammensetzung nach Anspruch 32, wobei das Verhältnis von Aluminiumoxid zu Bindemittel, bezogen auf das Gewicht, mindestens 7:1 beträgt.

34. Beschichtungszusammensetzung nach Anspruch 33, wobei das Verhältnis von Aluminiumoxid zu Bindemittel, bezogen auf das Gewicht, mindestens 9:1 beträgt.

35. Beschichtungszusammensetzung nach einem der Ansprüche 24 - 34, wobei die hochdispersen Aluminiumoxidpartikel eine Oberfläche von 40 - 60 m² / g aufweisen.

36. Verfahren zur Herstellung einer Beschichtungszusammensetzung, wobei das Verfahren umfasst:
Bereitstellen einer kolloidal stabilen Dispersion, die Wasser und hochdisperse Aluminiumoxidpartikel umfasst, wobei die hochdispersen Aluminiumoxidpartikel Aggregate von Primärpartikeln sind, die eine Oberfläche von 30 - 80 m² / g aufweisen und der Feststoffgehalt der hochdispersen Aluminiumoxidpartikel in der Dispersion 20 - 50 Gew. % beträgt;
Zugeben eines Bindemittels und ggf. Verdünnen der kolloidal stabilen Dispersion, bis ein gewünschtes Verhältnis von Pigment zu Bindemittel und Gesamtfeststoffgehalt erhalten wird; und
ggf. Einstellen des pH mit einer geeigneten Säure oder Base.

37. Verfahren nach Anspruch 36, wobei die Aggregate einen mittleren Durchmesser von weniger als 1 µm aufweisen.

38. Verfahren nach Anspruch 37, wobei die Aggregate einen mittleren Durchmesser von 80 - 300 nm aufweisen.

39. Verfahren nach Anspruch 38, wobei die Aggregate einen mittleren Durchmesser von 100 - 200 nm aufweisen.

40. Verfahren nach einem der Ansprüche 36 - 39, wobei die Primärpartikel einen mittleren Durchmesser von 1 - 100 nm aufweisen.

41. Verfahren nach Anspruch 40, wobei die Primärpartikel einen mittleren Durchmesser von 1 - 80 nm aufweisen.

42. Verfahren nach Anspruch 41, wobei die Primärpartikel einen mittleren Durchmesser von 1 - 50 nm aufweisen.

43. Verfahren nach Anspruch 42, wobei die Primärpartikel einen mittleren Durchmesser von 5 - 40 nm aufweisen.

44. Verfahren nach einem der Ansprüche 36 - 43, wobei das Verhältnis von Aluminiumoxid zu Bindemittel, bezogen auf das Gewicht, mindestens 2:1 beträgt.

45. Verfahren nach Anspruch 44, wobei das Verhältnis von Aluminiumoxid zu Bindemittel, bezogen auf das Gewicht, mindestens 7:1 beträgt.

46. Verfahren nach Anspruch 45, wobei das Verhältnis von Aluminiumoxid zu Bindemittel, bezogen auf das Gewicht, mindestens 9:1 beträgt.

47. Verfahren nach einem der Ansprüche 36-46, wobei die hochdispersen Aluminiumoxidpartikel eine Oberfläche von 40- 60 m² / g aufweisen.

48. Verfahren nach einem der Ansprüche 36 - 47, wobei der Feststoffgehalt der hochdispersen Aluminiumoxidpartikel in der kolloidal stabilen Dispersion 30 - 50 Gew. % beträgt.

49. Verfahren nach einem der Ansprüche 36 - 48, wobei das Zeta-Potential der Aluminiumoxidpartikel der kolloidal stabilen Dispersion mindestens + 20 mV beträgt.

50. Verfahren nach einem der Ansprüche 36 - 49, wobei der pH der kolloidal stabilen Dispersion 3 - 5 beträgt.

51. Verfahren nach einem der Ansprüche 36 - 50, wobei die Dichte der kolloidal stabilen Dispersion 1 - 2 kg / I beträgt.

52. Verfahren nach einem der Ansprüche 36 - 51, wobei die scheinbare Dichte der kolloidal stabilen Dispersion weniger als 0,02 Pa.s (20 cp) beträgt, gemessen in einem Herkules ® High-Shear Viskometer bei 4400 UPM, FF Bob Messgeometrie.

53. Verfahren nach einem der Ansprüche 36 - 52, wobei die Viskosität der kolloidal stabilen Dispersion weniger als 0,1 Pa.s (100 cp) beträgt, gemessen in einem Brookfield Model RV Viskometer, Spindel Nummer 1, nach 30 Sekunden bei 60 UPM)

54. Beschichtungszusammensetzung, erhältlich nach dem Verfahren nach einem der Ansprüche 36 - 53.

55. Verfahren zur Herstellung eines Tintenstrahlaufzeichnungsmediums, wobei das Verfahren umfasst:
Bereitstellen eines Substrats;
Beschichten des Substrats mit der Beschichtungszusammensetzung nach einem der Ansprüche 24 - 35, um ein Substrat herzustellen, das mit einer bestimmten Beschichtung beschichtet ist;
ggf. Kalandrieren des beschichteten Substrats; und
Trocken des beschichteten Substrats.

56. Verfahren zur Herstellung eines Tintenstrahlaufzeichnungsmediums, wobei das Verfahren umfasst:
Bereitstellen eines Substrats;
Beschichten des Substrats mit der Beschichtungszusammensetzung nach Anspruch 54, um ein Substrat herzustellen, das mit einer Beschichtung beschichtet ist;
ggf. Kalandrieren des beschichteten Substrats; und
Trocknen des beschichteten Substrats.

57. Tintenstrahlaufzeichnungsmedium, erhältlich nach einem Verfahren nach den Ansprüchen 55 oder 56.

## Revendications

1. Support d'enregistrement à jet d'encre comprenant un substrat sur lequel se trouve un revêtement brillant, le revêtement brillant comprenant des particules d'alumine sublimées et un liant, le revêtement brillant ayant un brillant spéculaire à 75° de 15 % ou plus, et les particules d'alumine sublimées sont des agrégats de particules primaires et présentent une surface spécifique de 30 à 80 m²/g.

2. Support d'enregistrement à jet d'encre selon la revendication 1, dans lequel le substrat comprend un polymère ou du papier cellulose.

3. Support d'enregistrement à jet d'encre selon la revendication 1 ou 2, dans lequel le substrat comprend du poly(téréphtalate d'éthylène).

4. Support d'enregistrement à jet d'encre selon l'une quelconque des revendications 1 à 3, dans lequel les agrégats ont un diamètre moyen inférieur à 1 µm.

5. Support d'enregistrement à jet d'encre selon la revendication 4, dans lequel les agrégats ont un diamètre moyen de 80 à 300 nm.

6. Support d'enregistrement à jet d'encre selon la revendication 5, dans lequel les agrégats ont un diamètre moyen de 100 à 200 nm.

7. Support d'enregistrement à jet d'encre selon la revendication 4, dans lequel au moins environ 80 % des agrégats ont un diamètre inférieur à 1 µm.

8. Support d'enregistrement à jet d'encre selon la revendication 7, dans lequel au moins environ 90 % des agrégats ont un diamètre inférieur à 1 µm.

9. Support d'enregistrement à jet d'encre selon l'une quelconque des revendications 1 à 8, dans lequel les particules primaires ont un diamètre moyen de 1 à 100 nm.

10. Support d'enregistrement à jet d'encre selon la revendication 9, dans lequel les particules primaires ont un diamètre moyen de 1 à 80 nm.

11. Support d'enregistrement à jet d'encre selon la revendication 10, dans lequel les particules primaires ont un diamètre moyen de 1 à 50 nm.

12. Support d'enregistrement à jet d'encre selon la revendication 11, dans lequel les particules primaires ont un diamètre moyen de 5 à 40 nm.

13. Support d'enregistrement à jet d'encre selon la revendication 9, dans lequel au moins environ 80 % des particules primaires ont un diamètre de 1 à 100 nm.

14. Support d'enregistrement à jet d'encre selon la revendication 10, dans lequel au moins environ 80 % des particules primaires ont un diamètre de 1 à 80 nm.

15. Support d'enregistrement à jet d'encre selon la revendication 11, dans lequel au moins environ 80 % des particules primaires ont un diamètre de 1 à 50 nm.

16. Support d'enregistrement à jet d'encre selon la revendication 12, dans lequel au moins environ 80 % des particules primaires ont un diamètre de 5 à 40 nm.

17. Support d'enregistrement à jet d'encre selon l'une quelconque des revendications 1 à 16, dans lequel le rapport alumine sur liant est d'au moins 2 : 1 en poids.

18. Support d'enregistrement à jet d'encre selon la revendication 17, dans lequel le rapport alumine sur liant est de 7 : 1 en poids ou plus.

19. Support d'enregistrement à jet d'encre selon la revendication 18, dans lequel le rapport alumine sur liant est de 9 : 1 en poids ou plus.

20. Support d'enregistrement à jet d'encre selon l'une quelconque des revendications 1 à 19, dans lequel les particules d'alumine sublimées ont une surface spécifique de 40 à 60 m²/g.

21. Support d'enregistrement à jet d'encre selon l'une quelconque des revendications 1 à 20, dans lequel le revêtement brillant a un brillant spéculaire à 75° de 65 % ou plus.

22. Support d'enregistrement à jet d'encre selon l'une quelconque des revendications 1 à 21, dans lequel le substrat est non poreux et le revêtement brillant a un volume d'intrusion de mercure total de 0,3 mL/g ou plus.

23. Support d'enregistrement à jet d'encre selon la revendication 22, dans lequel le revêtement brillant a un volume d'intrusion de mercure total de 0,8 mL/g ou plus.

24. Composition de revêtement comprenant des particules d'alumine sublimées et un liant, les particules d'alumine sublimées étant des agrégats de particules principales et ayant une surface spécifique de 30 à 80 m²/g et la teneur en solides des particules d'alumine sublimées dans la composition étant de 10 à 50 % en poids.

25. Composition de revêtement selon la revendication 24, dans laquelle les agrégats ont un diamètre moyen inférieur à 1 µm.

26. Composition de revêtement selon la revendication 25, dans laquelle les agrégats ont un diamètre moyen de 80 à 300 nm.

27. Composition de revêtement selon la revendication 26, dans laquelle les agrégats ont un diamètre moyen de 100 à 200 nm.

28. Composition de revêtement selon l'une quelconque des revendications 24 à 27, dans laquelle les particules primaires ont un diamètre moyen de 1 à 100 nm.

29. Composition de revêtement selon la revendication 28, dans laquelle les particules primaires ont un diamètre moyen de 1 à 80 nm.

30. Composition de revêtement selon la revendication 29, dans laquelle les particules primaires ont un diamètre moyen de 1 à 50 nm.

31. Composition de revêtement selon la revendication 30, dans laquelle les particules primaires ont un diamètre moyen de 5 à 40 nm.

32. Composition de revêtement selon l'une quelconque des revendications 24 à 31, dans laquelle le rapport alumine sur liant est d'au moins 2 : 1 en poids.

33. Composition de revêtement selon la revendication 32, dans laquelle le rapport alumine sur liant est d'au moins 7 : 1 en poids.

34. Composition de revêtement selon la revendication 33, dans laquelle le rapport alumine sur liant est d'au moins 9 : 1 en poids.

35. Composition de revêtement selon l'une quelconque des revendications 24 à 34, dans laquelle les particules d'alumine sublimées ont une surface spécifique de 40 à 60 m²/g.

36. Procédé de préparation d'une composition de revêtement, le procédé comprenant :
la formation d'une dispersion colloïdalement stable comprenant de l'eau et des particules d'alumine sublimées, les particules d'alumine sublimées étant des agrégats de particules primaires, ayant une surface spécifique de 30 à 80 m²/g et la teneur en solides des particules d'alumine sublimées dans la dispersion étant de 20 à 50 % en poids ;
l'ajout d'un liant à la dispersion colloïdalement stable et facultativement, la dilution de celle-ci jusqu'à l'obtention d'un rapport pigment sur liant et d'une teneur en solides globale souhaités ; et
facultativement, l'ajustement du pH à l'aide d'un acide ou d'une base approprié.

37. Procédé selon la revendication 36, dans lequel les agrégats ont un diamètre moyen inférieur à 1 µm.

38. Procédé selon la revendication 37, dans lequel les agrégats ont un diamètre moyen de 80 à 300 µm.

39. Procédé selon la revendication 38, dans lequel les agrégats ont un diamètre moyen de 100 à 200 µm.

40. Procédé selon l'une quelconque des revendications 36 à 39, dans lequel les particules primaires ont un diamètre moyen de 1 à 100 nm.

41. Procédé selon la revendication 40, dans lequel les particules primaires ont un diamètre moyen de 1 à 80 nm.

42. Procédé selon la revendication 41, dans lequel les particules primaires ont un diamètre moyen de 1 à 50 nm.

43. Procédé selon la revendication 42, dans lequel les particules primaires ont un diamètre moyen de 5 à 40 nm.

44. Procédé selon l'une quelconque des revendications 36 à 43, dans lequel le rapport alumine sur liant est d'au moins 2 : 1 en poids.

45. Procédé selon la revendication 44, dans lequel le rapport alumine sur liant est d'au moins 7 : 1 en poids.

46. Procédé selon la revendication 45, dans lequel le rapport alumine sur liant est d'au moins 9 : 1 en poids.

47. Procédé selon l'une quelconque des revendications 36 à 46, dans lequel les particules d'alumine sublimées ont une surface spécifique de 40 à 60 m²/g.

48. Procédé selon l'une quelconque des revendications 36 à 47, dans lequel la teneur en solides des particules d'alumine sublimées dans la dispersion colloïdalement stable est de 30 à 50 % en poids.

49. Procédé selon l'une quelconque des revendications 36 à 48, dans lequel le potentiel zêta des particules d'alumine dans la dispersion colloïdalement stable est d'au moins +20 mV.

50. Procédé selon l'une quelconque des revendications 36 à 49, dans lequel le pH de la dispersion colloïdalement stable est de 3 à 5.

51. Procédé selon l'une quelconque des revendications 36 à 50, dans lequel la masse volumique spécifique de la dispersion colloïdalement stable est de 1 à 2 kg/L.

52. Procédé selon l'une quelconque des revendications 36 à 51, dans lequel la viscosité apparente de la dispersion colloïdalement stable est inférieure à 0,02 Pa.s (20 cp) telle que mesurée dans un viscosimètre à fort taux de cisaillement Hercule® à 4 400 tr/min, géométrie de mesure FF Bob.

53. Procédé selon l'une quelconque des revendications 36 à 52, dans lequel la viscosité de la dispersion colloïdalement stable est inférieure à 0,1 Pa.s (100 cp) telle que mesurée dans un viscosimètre Brookfield modèle RV, tige n° 1, après 30 secondes à 60 tr/min.

54. Composition de revêtement pouvant être obtenue par le procédé selon l'une quelconque des revendications 36 à 53.

55. Procédé de préparation d'un support d'enregistrement à jet d'encre, le procédé comprenant :
la formation d'un substrat ;
le revêtement du substrat avec la composition de revêtement selon l'une quelconque des revendications 24 à 35 pour produire un substrat revêtu avec un revêtement ;
facultativement le calandrage du substrat revêtu ; et
le séchage du substrat revêtu.

56. Procédé de préparation d'un support d'enregistrement à jet d'encre, le procédé comprenant :
la formation d'un substrat ;
le revêtement du substrat avec la composition de revêtement selon la revendication 54 pour produire un substrat revêtu avec un revêtement ;
facultativement le calandrage du substrat revêtu ; et
le séchage du substrat revêtu.

57. Support d'enregistrement à jet d'encre pouvant être obtenu par le procédé de la revendication 55 ou 56.
